

## UNITED STATES PATENT OFFICE

2,000,656

PROCESS FOR FLOATING URANIUM ORES  
PARTICULARLY CARNOTITEHarry Howard Armstrong and Arthur Burley  
Menefee, Los Angeles, Calif.No Drawing. Application January 30, 1933,  
Serial No. 654,238

17 Claims. (Cl. 209—166)

Up to the present, the flotation of carnotite has been an operation of extreme difficulty or impossibility. As late as 1930, the U. S. Bureau of Mines in its pamphlet "Reports of Investigations" No. 3057, states on page 4: "The usual methods for concentrating ores, such as flotation or tabling, have not been successfully applied to carnotites."

The object of this invention is to provide a process whereby carnotite and other uranium ores including substantially all of its uranium and radium values, can be cleanly separated from its siliceous gangue by flotation. Torbernite, autunite and the uraninites are other ores which may be treated by our process.

The first step in the process is to grind or crush the carnotite finely, say to 60 mesh or finer. The crushing may be done wet or dry.

The second step is to treat the crushed ore which has been made into a thin pulp, usually with soft water, then with either a dilute solution of a sodium or potassium soap or to agitate the pulp with a fatty acid, such as lauric, or do both. In this step the carnotite particles are contacted with the soap or fatty acid or both and the effect is, that they are conditioned and will separate from the gangue under the subsequent treatment. This process of contacting may be carried out in the wet grinding of the ore or in an agitator or conditioning apparatus or in the flotation machine itself.

The third step is to run the pulp to any conventional type flotation machine, the exact condition of dilution being of no great importance. From one part ore to four parts water up to one part ore to twelve parts water have been used for dilution in obtaining satisfactory experimental results. A frothing agent is now usually added, for example, pine oil or any other conventional frother, if the soap is not sufficient to produce the froth required. The quantity is left to the discretion of the operator. Also before the actual flotation is done, there is added for each ton of ore being treated, one half pound or more of a soluble lead salt, preferably lead acetate, the function of which is probably that of a selective promoter, as it permits the minerals containing uranium, such as carnotite to float selectively from the gangue minerals.

The pulp in the machine is floated according to whatever technique the machine demands, usually mechanical or air agitation. The uranium material is carried up to the top in a froth or scum and is either overflowed or removed by

scraping off, thus separating it from the gangue materials.

The froth from the first or rougher cell or unit is usually recleaned by floating again in other cells according to ordinary practice. The final concentrate from a uranium ore like carnotite carrying from one to three percent  $U_3O_8$  results in product containing from 8% to 30%  $U_3O_8$  by weight. With some ores the addition of some silica depressant such as sodium silicate is required to bring up the concentrate to these high contents of uranium. From one half pound to five pounds is the range of depressant per ton of ore. It may be used only in the cleaning or final operation or it may be used in all the cell steps. The amounts of the reagents required vary widely according to the uranium and other component parts of the ore, especially the gangue materials and in particular calcium materials and finally in the degree of softness of the water. As an example, a typical carnotite ore is one varying in the  $U_3O_8$  content from 1% to 5% and the usual range of reagents will be as follows:

A. Soap from 0.2 lb. per ton to 10 lbs. per ton. Fatty acids from 0.5 lb. per ton to 6 lbs. per ton.

The fatty acids which are solids at normal temperatures, for example stearic, lauric or palmitic, are dissolved in solvents, such as kerosene, gasoline, acetone, benzol, etc. In solution they may be handled satisfactorily as flotation reagents.

B. Soluble lead salts such as lead acetate or lead nitrate are used in aqueous solutions in quantities from 0.5 lb. to 8 lbs. per ton of ore.

There are several additional steps that we may include in our process to render difficult ores more amenable to treatment. These are herewith given, altho it is to be understood that they are not always essential. They are:

1. Preliminary roasting of the ore with free access of air to rid the ore of carbon content.

2. Contacting the ore with dilute sulfuric acid (0.25% to 1.0% concentration) after pulping, to convert the Ra, Ba, and Pb present to insoluble sulfates and to neutralize excessive alkalinity of the ore and then removing excess acid.

3. If the ore pulp is acid, sodium carbonate or sodium hydroxide (0.25% to 1%) may be used to neutralize it thus rendering unnecessary the subsequent use of larger quantities of more expensive reagents such as soaps.

The amount of neutralization or softening to be done bears a rough relation to the  $U_3O_8$  content of the ore. Low grade ores usually require more neutralization than high grade ores for the reason that they contain more gangue. It is the

gangue materials (except  $\text{SiO}_2$ ) that give the ore either its alkaline or acid character. The adaptation of the amount of neutralization or softening of the water or the pulp to the  $\text{U}_3\text{O}_8$  content of the ore lies distinctly within our invention. In any case where an ore is encountered that gives a pulp outside the range of pH slightly under 7 to 8 inclusive, neutralization or softening is usually practiced. In other words, the flotation process will proceed with the best results, when the pulp is neutral or slightly alkaline and it lies within the scope of the invention to make it so.

We claim as our invention:

- 15 1. The process of floating uranium ores which comprises pulping a uranium ore, adjusting the pH of the pulp to nearly 7 to 8, contacting the pulp with a dilute alkali soap solution and then subjecting said pulp to flotation procedure in the presence of a water-soluble lead salt.
- 20 2. A process according to claim 1 in which the pulp of a uranium ore is subjected to flotation in the presence of a frothing agent in addition to the soap.
- 25 3. A process according to claim 1 in which the pulp of a uranium ore is subjected to flotation in the presence of a silica depressant.
- 30 4. A process according to claim 1 in which the uranium ore is carnotite.
- 35 5. A process according to claim 1 in which the pulp is acidified with  $\text{H}_2\text{SO}_4$  before adjustment of the pH to nearly 7 to 8.
- 40 6. The process of floating uranium ore which comprises pulping the ore with water, adjusting the pH of the pulp to the neighborhood of 7 to 8, contacting the pulp with an alkali metal soap solution of 0.25% to 1% strength, subjecting the so-prepared pulp to flotation procedure in the presence of a water soluble lead salt and removing the  $\text{U}_3\text{O}_8$  containing froth thereby produced.
- 45 7. A process according to claim 6 in which pine oil is added to the pulp prior to flotation.
8. A process according to claim 6 in which sodium silicate is added to the pulp before subjecting the latter to flotation procedure.
- 45 9. A process according to claim 6 in which the uranium ore is carnotite.

10. A process according to claim 6 in which the water soluble lead salt is lead acetate.

11. The process of recovering a  $\text{U}_3\text{O}_8$  concentrate by flotation which comprises pulping a uranium ore with water, rendering the  $\text{Ra}$ ,  $\text{Ba}$  and  $\text{Pb}$  salts in the pulp water insoluble, adjusting the pH of the pulp to the neighborhood of 7 to 8, contacting the pulp with a dilute alkali metal soap solution of not more than 1% strength, subjecting the so-prepared pulp to flotation procedure in the presence of a soluble lead salt in the proportion of 0.5 lb. to 8 lbs. per ton of ore and mechanically removing the  $\text{U}_3\text{O}_8$  containing froth so produced. 10

12. A process according to claim 11 in which the uranium ore is carnotite.

13. A process according to claim 11 in which the flotation is conducted in the presence of sodium silicate.

14. A process according to claim 11 in which the lead salt is lead acetate.

15. A process according to claim 11 in which the soluble lead salt is lead nitrate.

16. A process according to claim 11 in which the  $\text{Ra}$ ,  $\text{Ba}$  and  $\text{Pb}$  salts are rendered insoluble 25 by being converted to their sulfates by preliminarily contacting the finely ground ore with dilute sulfuric acid.

17. The process of preparing a  $\text{U}_3\text{O}_8$  concentrate containing from 8% to 30%  $\text{U}_3\text{O}_8$  by weight 30 which comprises pulping a uranium ore containing from 0.5% to 3%  $\text{U}_3\text{O}_8$  selected from the group comprising carnotite, torbernite, autunite and the uraninites, adjusting the pH of the pulp to the neighborhood of neutrality to slightly alkaline, contacting the so-prepared pulp with an alkali metal soap solution of from 0.25% to 1.0% strength, adding a water soluble lead salt in the proportion of from 0.5 lb. to 8 lbs. per ton of ore, 40 subjecting the mixture to agitation to produce a  $\text{U}_3\text{O}_8$  containing froth and then separating the said froth from the pulp and the gangue. 45

HARRY HOWARD ARMSTRONG. 45  
ARTHUR BURLEY MENEFEE.